# EUROPEAN PATENT SPECIFICATION

(11) **EP 2 931 929 B1**
(45) Date of publication and mention of the grant of the patent: **14.06.2017**
(21) Application number: 13824341.5
(22) Date of filing: 16.12.2013
(51) Int. Cl.: C22C 9/04, A44C 27/00

(54) **ALLOY FOR THE PRODUCTION OF JEWELS**
LEGIERUNG ZUR HERSTELLUNG VON JUWELEN
ALLIAGE POUR LA PRODUCTION DE BIJOUX

(30) Priority: 17.12.2012 IT VI20120335
(43) Date of publication of application: 21.10.2015
(73) Proprietor: CRIERI S.R.L., 15048 Valenza (AL) (IT)
(72) Inventor: GARFARINO, Mario, I-36057 Arcugnano (VI) (IT)
(74) Representative: Bonini, Ercole
(86) International application number: PCT/IB2013/002810
(87) International publication number: WO 2014/096938

(56) References cited:
- DE-A1-102005 045 477
- GB-A- 2 041 974
- JP-A- 55 125 246
- JP-A- 56 095 491
- KR-A- 20120 080 810
- KR-A- 20120 081 724
- KR-A- 20120 083 184
- KR-A- 20120 085 127
- US-A1- 2009 317 291
- US-A1- 2009 317 292

## Description

### Technical field of the invention

The invention concerns an alloy for the production of jewels, in particular precious jewels or trinkets. The invention concerns jewels, produced with this alloy.

### State of the art

In the market of jewellery and costume jewellery a large number of gold alloys or alloys of other precious metals, like for example platinum, are known and used to make jewels. Gold and platinum are metals that do not oxidize easily but they are very expensive. The weight of gold and platinum is relatively high, which limits the size that can be reasonably obtained for the jewels, in particular in the case of earrings.

In order to be able to offer jewels also at reasonable prices, the market of costume jewellery has developed several alloys that are based on copper and zinc, components of brass, and that are less expensive than gold alloys but pose several drawbacks.

In order to prevent the oxidation of the alloy and therefore the alteration of its gilded appearance, it is necessary to coat the item, for example with a golden layer, by means of a plating process carried out using galvanising methods.

This layer, however, is subject to wear. Owing to the oxidation processes, in most cases the alloys that replace the traditional gold alloys do not maintain their gilded appearance over time and need to be frequently cleaned or plated with alloys having a high gold content. Moreover, often these alloys do not imitate the precious metal and its alloys perfectly in terms of external appearance, that is, in terms of colour and degree of brightness.

The US patent application US 2009/0317291 A1 describes alloys for jewels with low gold carat rating comprising silver, copper and zinc as main components in addition to gold. The application explains that the alloys with less than 4 carats in gold can present oxidation problems with consequent fogging of the alloy.

### Presentation of the invention

The object of the present invention is to provide an improved alloy that overcomes the drawbacks listed above. The object of the present invention is mainly to propose an alloy with a low precious metal carat rating that, in addition to not oxidizing easily and having good workability, imitates the aspect and the brightness of precious metals and their alloys.

The objects mentioned above and others that are highlighted in greater detail below are achieved by an alloy for the production of jewels according to the claims. It is to be understood that the alloys described herein can always contain other elements, meaning elements that are not listed as components that make up the alloy, in the form of inevitable traces. These traces derive from impurities present in the raw materials or are residues of auxiliary materials used during the production or processing of the alloy. In this case, the remaining percentage needed to reach 100% by weight is constituted by copper and inevitable impurities. Advantageously, the traces are present in total quantities not exceeding 0.2% by weight.

The addition of metals such as gallium and/or indium helps lower the melting point of the alloy. In order to affect the fluidity of the molten material and the suitability of the material for precision casting, forming (in this case silicon-free alloys are preferably used) or welding (in this case indium should be preferably added), the expert in the art, thanks to his/her general knowledge of the matter, changes the percentages of the auxiliary components. The variation in the content of copper compared to metals with a silvery colouring, like for example zinc, silver and palladium, makes it possible to obtain different colours of the alloy, varying from red or rose through gold yellow until obtaining hues that correspond to those known for white gold.

Surprisingly, the low carat rating of gold, platinum and palladium, respectively, makes it possible to produce alloys that imitate the colours of the respective precious metals or their alloys while at the same time showing a high degree of brightness.

Moreover, the alloy is very elastic, easy to clean, polish and machine and has good lapping values, partly better than those of other alloys with higher carat rating.

According to an advantageous embodiment of the invention, the alloy does not contain iridium, germanium, silicon, osmium, tin, indium and gallium as elements that make up the alloy. As explained above, the alloy, in any case, can contain these elements within the group consisting of traces of other elements.

The variant embodiments described below are the compositions that in the search for economic alloys with low precious metal carat rating have proved to be particularly suited to be used to make trinkets, because they do not oxidize easily, are easy to machine and shiny, and imitate the shades of alloys with high carat rating.

A much preferred variant embodiment of the invention concerns an alloy comprising 4.17% by weight of a metal or a combination of metals selected among a) platinum, b) palladium, and c) platinum and palladium.

Preferred quantities of gold are 0.2% by weight - 3.5% by weight.

Other preferred ranges in the alloy are 0.5-1% gold by weight; 1.1-2.5% gold by weight or 2.6-3.5% gold by weight.

Preferably, in an alloy according to the invention iridium, germanium, silicon, osmium, tin, indium and gallium are not present, silver is present in quantities included between 8 and 10% by weight and zinc is present in quantities included between 15 and 19% by weight. Even more preferably, the quantity of silver corresponds to 8.8-9.2% by weight, the quantity of zinc to 16.8-17.2% by weight and the quantity of copper to 69.8-70.2% by weight.

A further preferred embodiment of the alloy according to the invention is constituted by an alloy comprising 4.17% by weight of a combination of gold, palladium and platinum, in which the three metals are present in equal quantities expressed in weight percentages.

In another preferred variant embodiment of the alloy according to the invention the alloy comprises 4.17% by weight of a combination of gold and palladium or of a combination of gold and platinum, in which the two metals are present in equal quantities expressed in weight percentages.

For the variant embodiments containing 4.17% by weight of the precious metals gold, platinum and/or palladium, the following is the preferred composition of the remaining 95.83% by weight: iridium, germanium, silicon, osmium, tin, indium and gallium are not present, silver is present in quantities included between 8 and 10% by weight, zinc is present in quantities included between 15 and 19% by weight, and the remaining percentage needed to reach 100% is constituted by copper. Even more preferably, the quantity of silver corresponds to 8.8-9.2% by weight and the quantity of zinc to 16.8-17.2% by weight.

A very advantageous variant embodiment of the invention concerns an alloy comprising 0.5% gold by weight and preferably at least 0.1% platinum by weight. Such an alloy is extraordinarily bright.

In a preferred variant embodiment, the alloy is consisting of 0.5% gold by weight; 12.5% silver and palladium by weight; 17% zinc by weight and 70% copper by weight wherein there is 0.1% platinum by weight which correspondingly partially replaces silver, palladium, zinc and/or copper, in accordance with the scope of the invention. The invention furthermore concerns a jewel, produced from an alloy according to the invention. Other possible items are, for example, coins, tableware, candle holders or other items of art handicraft.

It should be understood that the indicated values (their percentages by weight) always include also values that can be considered equivalent from the point of view of weighing accuracy and analysis of the individual components.

The alloy according to the invention is suited to be used in the processing cycles that are typical of the jewellery sector.

The invention achieves the object to provide an economic alloy with low carat rating of gold, platinum and palladium that, in addition to not oxidizing easily and having good workability, imitates the appearance of gold or its alloys with high carat rating and is considerably bright.

Further variant embodiments of the invention are described in the dependent claims. In the production stage, the alloy and the items manufactured therewith that are the subjects of the invention can be subjected to further modifications or construction variants that are not described herein. Said modifications or variants must all be considered protected by the present patent, provided that they fall within the scope of the claims expressed below.

### Description of preferred embodiments of the invention

The production of the alloy follows the methods known in the art for producing alloys containing gold, silver, brass, etc. which are not described herein for the sake of brevity.

The following table 1 lists some examples of embodiment of alloys according to the invention:

**Table 1**

| | gold | platinum | palladium | silver | zinc | copper |
|---|---|---|---|---|---|---|
| | [% by wt.] | [% by wt.] | [% by wt.] | [% by wt.] | [% by wt.] | [% by wt.] |
| Ex. 1 | 0,5 | 0 | 12,5 | | 17 | 70 |
| Ex. 2 | 0,5 | 0,1 | 0 | 12,4 | 17 | 70 |
| Ex. 3 | 1,39 | 1,39 | 1,39 | 8,83 | 17 | 70 |
| Ex. 4 | 2,09 | 2,09 | 0 | 8,83 | 17 | 70 |
| Ex. 5 | 2,09 | 0 | 2,09 | 8,83 | 17 | 70 |
| Ex. 6 | 4.17 of which 0.2-3.5 gold | | | 8-10 | 15-19 | rest |
| Ex. 7 | 4.17 of which 0.5-1.0 gold | | | 8-10 | 15-19 | rest |
| Ex. 8 | 4.17 of which 1.1-2.5 gold | | | 8-10 | 15-19 | rest |
| Ex. 9 | 4.17 of which 2.6-3.5 gold | | | 8-10 | 15-19 | rest |

The palladium and silver content of Ex. 1 is according to the claims of the invention.

Possible inevitable traces of other elements have not been indicated.

## Claims

1. Alloy for the production of jewels, consisting of: 7-16% silver by weight; 15-36% zinc by weight; 4.17% by weight of a combination of metals selected among a) gold and platinum, b) gold and palladium, and c) gold, platinum and palladium; 0-0.5% by weight of one or more metals selected among iridium, germanium, silicon, osmium, tin, indium and gallium; the rest being constituted by copper and inevitable impurities, wherein the alloy comprises from 0.2% to 3.5% gold by weight, preferably 0.5-1 % gold by weight or 1.1-2.5% gold by weight or 2.6-3.5% gold by weight.

2. Alloy for the production of jewels, consisting of: 7-16% silver by weight; 15-36% zinc by weight; 0.1-4.17% by weight of a metal or a combination of metals selected among a) platinum, b) palladium, and c) platinum and palladium; 0-0.5% by weight of one or more metals selected among iridium, germanium, silicon, osmium, tin, indium and gallium; the rest being constituted by copper and inevitable impurities.

3. Alloy according to claim 2, **characterized in that** it comprises 4.17% by weight of a metal or a combination of metals selected among a) platinum, b) palladium, and c) platinum and palladium.

4. Alloy according to claim 1 or 3, **characterized in that** iridium, germanium, silicon, osmium, tin, indium and gallium are not present therein, and silver is present in quantities included between 8 and 10% by weight, and **in that** zinc is present in quantities included between 15 and 19% by weight.

5. Alloy according to any of the claims 1 or 4, **characterized in that** it comprises 4.17% by weight of a combination of gold, palladium and platinum, in which the three metals are present in equal quantities expressed as weight percentages.

6. Alloy according to any of the claims 1 or 4, **characterized in that** it comprises 4.17% by weight of a combination of gold and palladium or a combination of gold and platinum, in which the two metals are present in equal quantities expressed as weight percentages.

7. Alloy for the production of jewels, consisting of: 7-16% silver by weight; 15-36% zinc by weight; up to 4.17% by weight of a metal or a combination of metals selected among a) gold and platinum, b) gold and palladium, and c) gold, platinum and palladium; 0-0.5% by weight of one or more metals selected among iridium, germanium, silicon, osmium, tin, indium and gallium; the rest being constituted by copper and inevitable impurities wherein the alloy comprises 0.5% gold by weight and preferably at least 0.1 % platinum by weight.

8. Alloy according to claim 7, **characterized in that** it is consisting of 0.5% gold by weight; 12.5% silver and palladium by weight; 17% zinc by weight and 70% copper by weight, in which there is 0.1% platinum by weight that correspondingly partially replaces silver, palladium, zinc and/or copper.

9. Alloy according to anyone of the claims 1, 3 or 5-8, **characterized in that** the 0-0.5% by weight of one or more metals are selected among iridium, germanium, silicon and gallium.

10. Jewel produced from an alloy according to any of the preceding claims.

## Patentansprüche

1. Legierung für die Herstellung von Schmuckstücken, Folgendes umfassend: 7-16% Gewichtsanteil Silber; 15-36% Gewichtsanteil Zink; 4,17% Gewichtsanteil einer aus a) Gold und Platin, b) Gold und Palladium, und c) Gold, Platin und Palladium ausgewählten Metallkombination; 0-0,5% Gewichtsanteil eines oder mehrerer aus Iridium, Germanium, Silicium, Osmium, Zinn, Indium und Gallium ausgewählten Metalle; wobei der Rest aus Kupfer und unvermeidbaren Verunreinigungen besteht und wobei die Legierung 0,2% bis 3,5% Gewichtsanteil Gold umfasst, vorzugsweise 0,5-1% Gewichtsanteil Gold oder 1,1-2,5% Gewichtsanteil Gold oder 2,6-3,5% Gewichtsanteil Gold.

2. Legierung für die Herstellung von Schmuckstücken, Folgendes umfassend: 7-16% Gewichtsanteil Silber; 15-36% Gewichtsanteil Zink; 0,1-4,17% Gewichtsanteil eines aus a) Platin, b) Palladium und c) Platin und Palladium ausgewählten Metalls oder einer daraus ausgewählten Metallkombination; 0-0,5% Gewichtsanteil eines oder mehrerer aus Iridium, Germanium, Silicium, Osmium, Zinn, Indium und Gallium ausgewählten Metalle; wobei der Rest aus Kupfer und unvermeidbaren Verunreinigungen besteht.

3. Legierung gemäß Patentanspruch 2, **dadurch gekennzeichnet, dass** sie 4,17% Gewichtsanteil eines aus a) Platin, b) Palladium und c) Platin und Palladium ausgewählten Metalls oder einer daraus ausgewählten Metallkombination umfasst.

4. Legierung gemäß Patentanspruch 1 oder 3, **dadurch gekennzeichnet, dass** sie kein Iridium, Germanium, Silicium, Osmium, Zinn, Indium und Gallium enthält und Silber in Mengen zwischen 8 und 10% Gewichtsanteil enthalten ist, und dadurch, dass Zink in Mengen zwischen 15 und 19% Gewichtsanteil enthalten ist.

5. Legierung gemäß eines jeden der Patentansprüche 1 oder 4, **dadurch gekennzeichnet, dass** sie 4,17% Gewichtsanteil einer Kombination aus Gold, Palladium und Platin umfasst, in der die drei Metalle in gleichen, als Gewichtsanteile ausgedrückten Mengen enthalten sind.

6. Legierung gemäß eines jeden der Patentansprüche 1 oder 4, **dadurch gekennzeichnet, dass** sie 4,17% Gewichtsanteil einer Kombination aus Gold und Palladium oder einer Kombination aus Gold und Platin umfasst, in der die drei Metalle in gleichen, als Gewichtsanteile ausgedrückten Mengen enthalten sind.

7. Legierung für die Herstellung von Schmuckstücken, Folgendes umfassend: 7-16% Gewichtsanteil Silber; 15-36% Gewichtsanteil Zink; bis zu 4,17% Gewichtsanteil eines/einer aus a) Gold und Platin, b) Gold und Palladium, und c) Gold, Platin und Palladium ausgewählten Metalls/ Metallkombination; 0-0,5% Gewichtsanteil eines oder mehrerer aus Iridium, Germanium, Silicium, Osmium, Zinn, Indium und Gallium ausgewählten Metalle; wobei der Rest aus Kupfer und unvermeidbaren Verunreinigungen besteht, und wobei die Legierung 0,5% Gewichtsanteil Gold und vorzugsweise wenigstens 0,1% Gewichtsanteil Platin umfasst.

8. Legierung gemäß Patentanspruch 7, **dadurch gekennzeichnet, dass** sie zu 0,5% Gewichtsanteil aus Gold, zu 12,5% Gewichtsanteil aus Silber und Palladium, zu 17% Gewichtsanteil aus Zink und zu 70% Gewichtsanteil aus Kupfer besteht, in dem 0,1% Gewichtsanteil Platin vorhanden ist, das entsprechend teilweise Silber, Palladium, Zink und/oder Kupfer ersetzt.

9. Legierung gemäß eines jeden der Patentansprüche 1, 3 oder 5-8, **dadurch gekennzeichnet, dass** der Gewichtsanteil von 0-0,5% eines oder mehrerer Metalle aus Iridium, Germanium, Silicium und Gallium ausgewählt ist.

10. Aus einer Legierung gemäß eines jeden der vorstehenden Patentansprüche hergestelltes Schmuckstück.

## Revendications

1. Alliage pour la production de bijoux, constitué de: 7-16% en poids d'argent; 15-36% en poids de zinc; 4,17% en poids d'une combinaison de métaux choisis parmi a) or et platine, b) or et palladium et c) or, platine et palladium; 0-0,5% en poids d'un ou plusieurs métaux choisis parmi iridium, germanium, silicium, osmium, étain, indium et gallium; le reste étant constitué de cuivre et d'impuretés inévitables, où l'alliage comprend 0,2-3,5% en poids d'or, préférablement 0,5-1% en poids d'or ou 1,1-2,5% en poids d'or ou 2,6-3,5% en poids d'or.

2. Alliage pour la production de bijoux, constitué de: 7-16% en poids d'argent; 15-36% en poids de zinc; 0,1-4,17% en poids d'un métal ou une combinaison de métaux choisis parmi a) platine, b) palladium et c) platine et palladium; 0-0,5% en poids d'un ou plusieurs métaux choisis parmi iridium, germanium, silicium, osmium, étain, indium et gallium; le reste étant constitué de cuivre et d'impuretés inévitables.

3. Alliage selon la revendication 2, **caractérisé en ce qu'**il comprend 4,17% en poids d'un métal ou une combinaison de métaux choisis parmi a) platine, b) palladium et c) platine et palladium.

4. Alliage selon la revendication 1 ou 3, **caractérisé en ce qu'**iridium, germanium, silicium, osmium, étain, indium et gallium ne sont pas présents, que l'argent est présent en quantités comprises entre 8 et 10% en poids et que le zinc est présent en quantités comprises entre 15 et 19% en poids.

5. Alliage selon l'une quelconque des revendications 1 ou 4, **caractérisé en ce qu'**il comprend 4,17% en poids d'une combinaison d'or, palladium et platine, où les trois métaux sont présents en quantités égales exprimées en pourcentages de poids.

6. Alliage selon l'une quelconque des revendications 1 ou 4, **caractérisé en ce qu'**il comprend 4,17% en poids d'une combinaison d'or et palladium ou d'une combinaison d'or et platine, où les deux métaux sont présents en quantités égales exprimées en pourcentages de poids.

7. Alliage pour la production de bijoux, constitué de: 7-16% en poids d'argent; 15-36% en poids de zinc; jusqu'à 4,17% en poids d'un métal ou une combinaison de métaux choisis parmi a) or et platine, b) or et palladium et c) or, platine et palladium; 0-0,5% en poids d'un ou plusieurs métaux choisis parmi iridium, germanium, silicium, osmium, étain, indium et gallium; le reste étant constitué de cuivre et d'impuretés inévitables, où l'alliage comprend 0,5% en poids d'or et préférablement au moins 0,1% en poids de platine.

8. Alliage selon la revendication 7, **caractérisé en ce qu'**il est constitué de 0,5% en poids d'or; 12,5% en poids d'argent et palladium; 17% en poids de zinc et 70% en poids de cuivre, où 0,1% en poids de platine est présent, qui proportionnellement remplace partiellement l'argent, le palladium, le zinc et/ou le cuivre.

9. Alliage selon l'une quelconque des revendications 1, 3 ou de 5 à 8, **caractérisé en ce que** 0-0,5% en poids d'un ou plusieurs métaux sont choisis parmi iridium, germanium, silicium et gallium.

10. Bijou produit à partir d'un alliage selon l'une quelconque des revendications précédentes.
